

Patented July 3, 1934

1,965,513

# UNITED STATES PATENT OFFICE

1,965,513

## PROCESS FOR IMPROVING COAL MATERIAL

Apollo Ružička, Usti Nad Labem, Krasnobrezen-  
ska, Czechoslovakia

No Drawing. Application July 13, 1932, Serial  
No. 622,362. In Bulgaria August 21, 1931

1 Claim. (Cl. 34—24)

As is well known, the drying of many fuels of high water content, particularly the geologically recent varieties, such as, for example, brown coal or lignite, offers great difficulties owing to the colloidal properties of the same. Particularly great difficulties arise during the drying of lump brown coal and the coarser varieties thereof, which frequently crumble and disintegrate when the drying processes heretofore known are employed.

It is already known to heat brown coal up to the drying temperature for drying purposes by introducing steam under pressure directly on to the material to be dried, and then effecting evaporation of the moisture by releasing the pressure. The employment of this steam introduced directly on to the material to be dried is disadvantageous, since the heat is too rapidly and too suddenly transferred to the coal, with the result that the outer layers of each lump of coal are heated suddenly and partial evaporation of the moisture contained therein takes place, whilst on the other hand the interior layers do not partake of this rapid heating, and consequently pressure differences arise between the inner and outer layers of the coal, which cause a more or less deep-seated disintegration of the lumps.

These drawbacks are removed by the process which forms the subject matter of this invention, and which consists essentially in that the material, partially immersed in supplied water, is heated in the pressure container together with the supplied water to a temperature of 150—250° C. at a pressure of the saturated water vapour present which corresponds to this temperature, the heating being effected, when employing an external heating medium, e. g. flue gas, by merely heating the lower part of the container filled with supplied water or, when employing direct introduction of steam, by leading the latter merely into the lower part of the pressure container filled with the added water. In the former case the steam is merely formed from the supplied water, and in the latter case the steam introduced saturates itself only from the supplied water, so that in both cases the evaporation of the moisture contained in the coal, as well as the superheating of the water vapour, are prevented with certainty. The pressure in the container is thereupon released and as a result a solid product, substantially moisture-free and non-colloidal is obtained.

According to the invention, therefore, not only are the above-mentioned drawbacks practically completely removed, but also a gradual, readily regulable increase in the temperature and the

pressure, suitably adaptable to the properties of the coal to be dried, and therefore a gradual, uniformly increasing, non-detrimental heating of the material is ensured and the formation of vapour from the moisture contained in the coal is avoided as well as all superheating of the water vapours, both of which bring about the differences in tension between the inner and outer coal layers of each lump of coal. Furthermore, a not inconsiderable diminution in the ash and sulphur content is brought about, varying according to the properties of the coal.

A further substantial advantage of this process consists in the possibility of employing superheated steam, by which means the economy of the process can be raised considerably.

It has also been found that the very high pressure of the water vapours contained in the colloidal coal material is the main cause of the disintegration of the fuels during the drying of the same.

The water vapours can escape from the colloidal coal material only with difficulty, and break it up in the case of deep penetration if this colloidal property has not previously been removed, it being borne in mind that the consistency of the material is maintained. This is brought about by heating the part of the pressure container filled with a suitable quantity of supplied water, as a result of which this colloidal quality of the coal, and its capability of binding moisture, is destroyed. The quantity of water added to the fuel depends on the moisture content of the material and its physical properties, and also on the heating medium employed for the heating, and on the desired final temperature and the desired pressure, there being in no case any superheating of the water vapours in the container, that is to say, there must always be a quantity of supplied water left during the heating, as well as after the attainment of the final temperature, such that the conditions of saturated water vapour always prevail in the pressure container.

The height of the temperature depends on the properties of the material to be dried. Preferably the highest possible temperatures are employed, which, however, do not attain the decomposition temperature of the coal mass, i. e. they must not result in any deep-seated decomposition of the coal material.

The coal treated according to this process loses its colloidal quality and separates out the greater part of the moisture contained therein without any considerable decomposition taking place.

The product produced is solid, contains little moisture, and no longer absorbs considerable quantities of moisture, even after wetting.

What I claim is:—

- 5 A method of improving (drying) fuel material, such as brown coal, consisting in partially immersing the material in water, heating the wa-

ter and the portion of the fuel immersed therein at a temperature selected from the range 150–250° C. and under a pressure of the saturated water vapour present which corresponds to the selected temperature, and thereupon releasing the 80 pressure.

APOLLO RUŽIČKA.

10

85

15

90

20

95

25

100

30

105

35

110

40

115

45

120

50

125

55

130

60

135

65

140

70

145

75

150